

## UNITED STATES PATENT OFFICE

FRANK L. REMLEIN, OF NEW YORK, N. Y., ASSIGNOR TO E. I. DU PONT DE NEMOURS & COMPANY, OF WILMINGTON, DELAWARE, A CORPORATION OF DELAWARE

## VAT DYEING

No Drawing.

Application filed September 21, 1927. Serial No. 221,144.

This invention relates to a process of applying vat colors to materials such as cotton piece goods. More particularly it relates to a special method of developing the color on 5 the goods.

In the usual art of vat dyeing, particularly with heavy shades, it has been practically impossible satisfactorily to pad the material being dyed without supplementing the padding operation by passing the fabric through 10 a jigger. The dyestuff in the unreduced form is padded on the fabric, and the penetration of the dye into the fibres of the fabric is expedited by thereafter passing the 15 padded fabric through a jigger in which is maintained a reducing bath. Even for light shades it has been found convenient to pad the fabric with the reduced dyestuff and then 20 subject the padded fabric to a jigger, in which is maintained a reducing bath. The reduced dyestuff in either case is thereafter developed by oxidation in the usual manner. The two steps of padding and jigging have 25 heretofore been necessary because without them it has been impossible to obtain a proper penetration of the fibres of the fabric. When the attempt has been made to dye 30 the fabric in a single stage process, the fabric has not been uniformly dyed.

It is one object of this invention to carry out a process of vat color printing or dyeing in a single step in place of the two steps heretofore used. It is a further object to permit 35 single step dyeing with vat colors in heavy as well as light shades. It is a further object of the invention to carry out the dyeing in such a way as to develop the color on the goods and obtain dyeings which are faster 40 to soaping and rubbing than are the dyeings of previous processes. It is a still further object to carry out the dyeing process in a way more economical than has heretofore been possible. Further objects will be apparent 45 from the description.

The above objects are attained by reducing 50 the vat color to its leuco-compound and applying the leuco-compound directly to the goods, at the same time retarding the oxidation of the leuco-compound sufficiently to

allow penetration of the dye into the fiber of the goods.

As a specific example, given by way of illustration and not in limitation, the vat color is reduced to its leuco-compound in 55 the usual manner in a vat containing caustic soda, glue and hydrosulfite. Specifically 160 gallons of pad liquor are prepared by adding the following ingredients to a sufficient quantity of water:

|                                    |    |
|------------------------------------|----|
| 10 lbs Ponsol blue GD double paste | 60 |
| (Schultz No. 842)                  |    |
| 8 lbs. of sodium hydroxide         |    |
| 8 lbs. of sodium hydrosulfite      |    |
| 8 lbs. animal glue                 | 65 |

To this liquor is added one quart of an anthraquinone solution prepared by dissolving in three parts of water the following ingredients:

|                                 |  |
|---------------------------------|--|
| 1 part of anthraquinone         |  |
| 1/8 part of sodium hydroxide    |  |
| 1/4 part of sodium hydrosulfite |  |

The goods to be dyed are padded or passed 70 through this combined solution and from this padding the goods are passed directly to a suitable squeeze roll, the color being forced into the goods by squeezing. The color is then developed with steam by running the wet goods from the squeeze rolls directly on hot cans (which are merely cylindrical drums, the interiors of which are steam heated) before the color is oxidized to its insoluble state. The goods are then soaped 75 at the boil in the usual way to remove any loose dyestuff which may be deposited on the surface of the goods.

This method is more economical than previous methods in that it combines in one step 80 the impregnation of the goods and reduction of the dye. The resultant dyeings obtained are faster to soaping and running than those previously obtained by the usual methods. In the usual pad-jig method, the dyestuff is padded or applied to the goods in unreduced form and thereafter penetration 85 of the dyestuff is expedited by the use of a reducing bath in a jigger. The use of the jig method entails the passage of the goods 90

100

back and forth through the dye bath for some time to obtain the desired results. The dyeings obtained by the present method are remarkably good and are superior for vat colors in both light and heavy shades.

5 Anthraquinone has been used in textile printing previously but it has always been used to render the discharge whiter. It has not served in any way to produce a colored 10 textile. However, where in the past anthraquinone has been used to remove color, the present method entails the use of anthraquinone in a dyeing process.

15 The method described is applicable to substantially all vat colors but its principal importance lies in connection with the anthraquinone vats, since these are characterized by the fact that they oxidize very rapidly.

20 Various modifications may be made in the details of the process. It will be apparent 25 that other alkalies may be used in place of caustic soda and other suitable reducing agents may be used in place of sodium hydrosulfite, if desired. The reducing bath to which the anthraquinone is added apparently reduces the anthraquinone to anthranol, as shown in the following formulæ:

